



US006814815B2

(12) **United States Patent**  
**Voges**

(10) Patent No.: **US 6,814,815 B2**  
(45) Date of Patent: **Nov. 9, 2004**

(54) **METHOD OF REMOVING SCALE AND INHIBITING OXIDATION IN PROCESSED SHEET METAL**

(75) Inventor: **Kevin Voges**, Red Bud, IL (US)

(73) Assignee: **The Material Works, Ltd.**, Red Bud, IL (US)

(\*) Notice: Subject to any disclaimer, the term of this patent is extended or adjusted under 35 U.S.C. 154(b) by 0 days.

(21) Appl. No.: **10/408,732**

(22) Filed: **Apr. 7, 2003**

(65) **Prior Publication Data**

US 2004/0194804 A1 Oct. 7, 2004

(51) **Int. Cl.** <sup>7</sup> ..... **B08B 1/00**; B08B 1/02; B21B 45/04; B21B 45/06; B21C 43/04

(52) **U.S. Cl.** ..... **134/9**; 134/42; 134/6; 134/15; 72/40

(58) **Field of Search** ..... 134/6, 42; 72/40

(56) **References Cited**

U.S. PATENT DOCUMENTS

|             |         |              |
|-------------|---------|--------------|
| 2,318,432 A | 5/1943  | Stanier      |
| 2,449,507 A | 9/1948  | Pope         |
| 2,907,151 A | 10/1959 | Peterson     |
| 3,686,921 A | 8/1972  | Roper        |
| 3,722,251 A | 3/1973  | Withrow      |
| 3,753,522 A | 8/1973  | Voges        |
| 3,924,428 A | 12/1975 | Noe          |
| 4,312,325 A | 1/1982  | Voges et al. |
| 4,539,830 A | 9/1985  | Noe          |
| 4,751,838 A | 6/1988  | Voges        |
| 4,872,245 A | 10/1989 | Kawasaki     |
| 4,887,502 A | 12/1989 | Voges        |
| 4,982,593 A | 1/1991  | Holloway     |
| 5,077,887 A | 1/1992  | Holloway     |
| 5,181,411 A | 1/1993  | Holloway     |
| 5,579,658 A | 12/1996 | Noe          |
| 5,759,307 A | 6/1998  | Berger       |
| 5,820,704 A | 10/1998 | Veyer        |

|                |         |                    |
|----------------|---------|--------------------|
| 5,829,287 A    | 11/1998 | Noe                |
| 6,088,895 A    | 7/2000  | Nelson et al.      |
| 6,089,063 A    | 7/2000  | Noe et al.         |
| 6,205,830 B1   | 3/2001  | Voges              |
| 6,210,501 B1   | 4/2001  | Okano et al.       |
| 6,732,561 B2 * | 5/2004  | Voges ..... 72/161 |

FOREIGN PATENT DOCUMENTS

|    |           |         |
|----|-----------|---------|
| DE | 1452957   | 4/1963  |
| EP | 498038 A2 | 8/1992  |
| JP | 58-116902 | 7/1983  |
| SU | 0158862   | 11/1963 |

OTHER PUBLICATIONS

3M Scotch-Brite Product Brochure, 1993.  
Leveltek International, LLC website information, Circa 1999.

\* cited by examiner

Primary Examiner—Zeinab El-Arini

(74) Attorney, Agent, or Firm—Thompson Coburn, LLP

(57) **ABSTRACT**

A method of removing iron oxide scale from processed sheet metal, the method includes the steps of: providing a surface conditioning apparatus; and conditioning a surface of the processed sheet metal with the surface conditioning apparatus. In general, the iron oxide scale generally comprises three layers prior to surface conditioning: a wustite layer, a magnetite layer, and a hematite layer. The wustite layer is bonded to a base metal substrate of the processed sheet metal. The magnetite layer is bonded to the wustite layer, and the hematite layer is bonded to the magnetite layer. The surface conditioning apparatus has at least one surface conditioning member. The step of conditioning the surface of the processed sheet metal includes bringing the at least one surface conditioning member into engagement with the surface of the sheet metal. The surface conditioning member is brought into engagement with the surface in a manner to remove substantially all of the hematite and magnetite layers from the surface, and in a manner to remove some but not all of the wustite layer from the surface, so that a portion of the wustite layer remains bonded to the base metal substrate of the processed sheet metal after surface conditioning.

**17 Claims, 5 Drawing Sheets**





Fig. 1



Fig. 2



Fig. 3



Fig. 4



Fig. 5



Fig. 6



Fig. 7

## 1

**METHOD OF REMOVING SCALE AND  
INHIBITING OXIDATION IN PROCESSED  
SHEET METAL**

**FIELD OF THE INVENTION**

The present invention relates generally to methods for removing iron oxide scale from processed sheet metal and inhibiting further oxidation in the processed sheet metal. More particularly, the present invention relates to methods for removing iron oxide scale from the surfaces of processed sheet metal using a mechanical surface conditioning apparatus in a manner to inhibit further oxidation on the conditioned surfaces and to reduce surface roughness.

**BACKGROUND OF THE INVENTION**

Processed sheet metal has a wide variety of applications. For example, aircraft, automobiles, file cabinets and household appliances, to name only a few, contain sheet metal bodies or shells. The sheet metal is typically purchased directly from steel mills and/or steel service centers, but may be passed through intermediate processors (sometimes referred to as "toll" processors) before it is received by an original equipment manufacturer. Sheet metal is typically formed by hot rolling process and, if the gauge is thin enough, it is coiled for convenient transport and storage. During the hot rolling process, carbon steel typically reaches finishing temperatures well in excess of 1500° F. (815° C.). Once the hot rolling process is completed, the hot rolled steel is reduced to ambient temperature, typically by quenching in water, oil or polymer, as is well known in the art. As a result of reactions with oxygen in the air and moisture, an iron oxide layer (or "scale") is formed on the surface of hot rolled carbon steel while the steel is cooled. The rate at which the product is cooled, and the total temperature drop, will affect the amount and composition of scale that forms on the surface during the cooling process.

Iron has a complex oxide structure with  $\text{FeO}$  ("wustite") mechanically bonded to the base metal substrate, followed by a layer of  $\text{Fe}_3\text{O}_4$  ("magnetite") chemically bonded to the wustite, and then a layer of  $\text{Fe}_2\text{O}_3$  ("hematite") chemically bonded to the magnetite and which is exposed to the air. Oxidation tends to progress more rapidly at higher temperatures, such as those reached in a typical hot rolling process, resulting in the formation of wustite. The relative thickness of each of the distinct wustite, magnetite and hematite layers is related to the availability of free oxygen and iron as the hot rolled substrate cools. When cooled from finishing temperatures above 1058° F. (570° C.), the oxide layer will typically comprise at least 50% wustite, and will also comprise magnetite and hematite in layers, formed in that order from the substrate. Though a number of factors (e.g., quenching rate, base steel chemistry, available free oxygen, etc.) affect the relative thicknesses of wustite, magnetite and hematite, as well as the overall thickness of the oxide layer, research has shown that the overall thickness of the oxide layer (inclusive of all three of these layers) in hot rolled carbon steel will typically be about 0.5% of the total thickness of the steel sheet. Thus, for example, in  $\frac{3}{8}$ " hot rolled carbon steel, the overall thickness of the oxide layer will be about 0.002".

Various methods exist for flattening sheet metal and for conditioning the surfaces thereof. Flatness of sheet metal is important because virtually all stamping and blanking operations require a flat sheet. Good surface conditions are also important, especially in applications where the top and/or

## 2

bottom surfaces of the metal sheet will be painted or otherwise coated. For processed sheet metal that is to be painted or galvanized, current industry practice is to remove all evidence of oxide from the surface to be painted or galvanized. With respect to painted surfaces, removing all evidence of oxide before painting ensures optimum adhesion, flexibility, and corrosion resistance of the intended paint coating layer. With respect to galvanizing, removing all evidence of oxide before coating allows a sufficient chemical bond of zinc to base metal.

The most common method of removing all oxide from the surface of hot rolled sheet metal before coating is a process known as "pickle and oil." In this process, the steel (already cooled to ambient temperature) is uncoiled and pulled through a bath of hydrochloric acid (typically about 30% hydrochloric acid and 70% water) to chemically remove the scale. Then, after the scale has been removed, the steel is washed, dried, and immediately "oiled" to protect it from rust damage. The oil provides an air barrier to shield the bare metal from exposure to air and moisture. It is critical that the metal be oiled immediately after the pickling process, as the bare metal will begin to oxidize very quickly when exposed to air and moisture. The "pickle and oil" process is effective in removing substantially all of the oxide layer, including the tightly bonded wustite layer, and results in a surface that is suitable for most coating applications. However, the "pickle and oil" process has a number of disadvantages. For example, the oil applied to the metal after pickling must be removed before coating, which is time consuming. Also, hydrochloric acid is an environmentally hazardous chemical, which has special storage and disposal restrictions. In addition, the oil coating interferes with some manufacturing processes, such as welding, causes stacked sheets to stick together, and gets into machine parts during manufacturing processes. Also, while the pickling process is effective at removing substantially all of the oxide layer, resulting in a surface that is suitable for most coating applications, the pickling agent (hydrochloric acid) tends to leave a clean but slightly coarse surface.

Thus, there is a need for an improved method of surface conditioning processed sheet metal, which removes enough scale from the surface to ensure optimum conditions for accepting coatings, which results in a smooth surface that is suitable for virtually all coating applications, which includes a means for inhibiting further oxidation prior to coating, and which is less expensive and troublesome than standard pickling and oiling.

**SUMMARY OF THE INVENTION**

It is therefore an object of the present invention to provide an improved method of removing iron oxide scale from processed sheet metal in a manner to ensure optimum surface conditions for accepting paint, galvanizing, or other coating. A related object is to provide an improved method of removing iron oxide scale from processed sheet metal, which results in a smooth surface that is suitable for virtually all coating applications. Another object is to provide an improved method of removing iron oxide scale from processed sheet metal in a manner that will inhibit further oxidation without the need to coat with oil. Still another general object is to provide an improved method of removing iron oxide scale from processed sheet metal, which is less expensive and troublesome than standard pickling and oiling.

The present invention includes methods of removing iron oxide scale from processed sheet metal, wherein the iron

oxide scale generally comprises three layers: a wustite layer, a magnetite layer, and a hematite layer. The wustite layer is bonded to a base metal substrate of the processed sheet metal. The magnetite layer is bonded to the wustite layer, and the hematite layer is bonded to the magnetite layer. In general, the methods comprise the steps of: providing a surface conditioning apparatus; and conditioning a surface of the processed sheet metal with the surface conditioning apparatus. The surface conditioning apparatus has at least one surface conditioning member. The step of conditioning the surface of the processed sheet metal includes bringing the at least one surface conditioning member into engagement with the surface in a manner to remove substantially all of the hematite layer and magnetite layer from the surface. Additionally, the surface conditioning member is brought into engagement with the surface in a manner to remove some but not all of the wustite layer from the surface, so that a portion of the wustite layer remains bonded to the base metal substrate of the processed sheet metal.

In another aspect of the invention, methods of removing iron oxide scale from processed sheet metal comprise the steps of: providing a surface conditioning apparatus having at least one rotating conditioning member; and conditioning a surface of the processed sheet metal with the surface conditioning apparatus. The step of conditioning the surface of the processed sheet metal includes bringing the at least one rotating conditioning member into engagement with the surface of the sheet metal. The rotating conditioning member is brought into engagement with the surface in a manner to remove some, but less than substantially all of the iron oxide scale from the surface so that a layer of oxide scale remains bonded to a base metal substrate of the processed sheet metal. Additionally, the rotating conditioning member is brought into engagement with the surface in a manner to reduce an arithmetic mean of distances of departure of peaks and valleys on the surface, measured from a mean center line, to less than 50 micro inches.

While the principal advantages and features of the present invention have been described above, a more complete and thorough understanding and appreciation of the invention may be attained by referring to the Figures and detailed description of the preferred embodiments, which follow.

#### BRIEF DESCRIPTION OF THE DRAWINGS

The accompanying Figures, which are incorporated in and form a part of the specification, illustrate exemplary embodiments of the present invention and, together with the description, serve to explain the principles of the invention.

FIG. 1 is a schematic representation of an in-line metal processing system incorporating a stretcher leveler and a surface conditioning apparatus of the type used in practicing the methods of the present invention;

FIG. 2 is a schematic representation of an in-line metal processing system comprising a tension leveler and a surface conditioning apparatus of the type used in practicing the methods of the present invention;

FIG. 3 is a schematic representation of another embodiment of an in-line metal processing system comprising a tension leveler and a surface conditioning apparatus of the type used in practicing the methods of the present invention;

FIG. 4 is a side elevational view of a portion of a surface conditioning apparatus of the type used in practicing the methods of the present invention;

FIG. 5 is a top plan view of a portion of a surface conditioning apparatus shown in FIG. 4;

FIG. 6 is a fragmented cross-sectional view of a length of processed sheet metal with layers of iron oxide scale, prior to surface conditioning according to the methods of the present invention; and

5 FIG. 7 is a fragmented cross-sectional view of a length of processed sheet metal after it has been surface conditioned according to the methods of the present invention.

Reference characters shown in these Figures correspond to reference characters used throughout the following 10 detailed description of the preferred embodiments.

#### DETAILED DESCRIPTION OF THE PREFERRED EMBODIMENTS

15 In performing the methods of the present invention, a surface conditioning apparatus, which will be described in detail hereinafter, may be used in conjunction with a number of different machines for flattening and leveling sheet metal, without departing from the scope of the present invention.

20 A surface conditioning apparatus of the type used in practicing the methods of the present invention is represented generally in FIG. 1 by the reference numeral 10. FIG. 1 is a schematic representation of an in-line metal processing system incorporating the surface conditioning apparatus 10, a stretcher leveler 12, and other components used therewith.

25 Viewed from left to right, FIG. 1 shows a coil of sheet metal 14 mounted on an upstream pay-off reel 16, a straightener 20, a take up pit 22, the stretcher leveler 12 and the surface conditioner 10. The straightener 20 is positioned just downstream of the reel 16 and includes a plurality of upper rollers 24 and lower rollers 26 having a relatively large diameter, which are positioned relative to one another to put a deep reverse bend in the sheet 30 sufficient to reverse coil set, as is well known in the art. The take up pit 22 is positioned just downstream of the straightener 20, and the stretcher leveler 12 is just downstream of the take up pit. The strip 30 is advanced incrementally through the stretcher leveler 12 for successive stretching operations, as is known in the art, and the take up pit 22 is positioned at the exit end of the

30 straightener 20 to take up slack in the continuously advancing strip 30 exiting the straightener as the strip 30 is advanced incrementally through the stretcher 12. As described more fully in U.S. Pat. No. 6,205,830 owned by the Applicant herein, the stretcher leveler 12 includes a

35 clamping mechanism that clamps down on a segment of the strip 30 and stretches that segment beyond its yield point to eliminate internal residual stresses, thereby leveling that segment. As explained in U.S. Pat. No. 6,205,830, stretcher leveling is a desirable method of leveling sheet metal

40 because it eliminates virtually all internal residual stresses and achieves superior flatness. With continued reference to FIG. 1, the surface conditioning apparatus 10 is positioned just downstream of the stretcher leveler 12. As shown in FIGS. 4 and 5, and as explained below in much more detail,

45 the surface conditioning apparatus 10 includes at least one mildly abrasive, rotating cleaning brush, which is brought into engagement with a surface of the sheet metal strip 30 to remove scale and other smut from the surface. Thus, FIG. 1 depicts one preferred environment for practicing the methods of the present invention, wherein the surface conditioning apparatus 10 is used in conjunction with a stretcher leveler 12.

50 However, again, it should be understood that, in performing the methods of the present invention, the surface conditioning apparatus 10 may be used in conjunction with a number of other machines for flattening and leveling sheet metal, without departing from the scope of the present invention.

55

60

65

FIG. 2 is a schematic representation of an in-line metal processing system wherein the surface conditioning apparatus **10** is used in conjunction with a tension leveler **40**. Viewed from left to right, FIG. 2 shows an upstream pay-off reel **42**, a coil **44** of sheet metal **46** mounted to the reel **42**, the tension leveling apparatus **40**, the surface conditioning apparatus **10**, and a downstream take-up reel **48**. In general, the tension leveling apparatus **40** comprises a drag bridle **50**, a leveler **52**, and a pull bridle **54**, as is known in the art. The drag bridle **50** includes a plurality of drag rollers **56**, which receive the metal sheet **46** from the upstream reel **42**. The pull bridle **54** includes a plurality of pull rollers **58**. The rollers of the drag and pull bridles **50** and **54** are powered, as is well known in the art, and rotate to advance the metal sheet through the tension leveler **40**. The leveler **52** is located between the drag and pull bridles **50** and **54** and includes a plurality of smaller radius leveling rollers **60**, which are offset from one another to impart bending stresses in the metal sheet **46** as the sheet is advanced therethrough. The pull rollers **58** of the pull bridle **54** turn slightly faster than the drag rollers **56** of the drag bridle **50**. Thus, the portion of the metal sheet **46** between the drag and pull bridles **50** and **54** is placed under a substantial tensile force. As is known in the art, this tensile force is preferably sufficient to stretch all fibers in the metal sheet **46** to exceed the material yield point as the metal sheet **46** is made to conform to the smaller radius of the leveling rollers **60** located between the drag and pull bridles **50** and **54**, as the metal sheet **46** passes through the leveling rollers **60**. With continued reference to FIG. 2, the surface conditioning apparatus **10** (explained below in much greater detail) is positioned just downstream of the tension leveler **40**. Thus, FIG. 2 depicts another preferred environment for practicing the methods of the present invention, wherein the surface conditioning apparatus **10** is used in conjunction with a tension leveler **40**. Tension leveling is also a preferred method of leveling sheet metal because of its ability to achieve an extremely flat condition of the sheet metal in a continuous coil-to-coil operation, substantially free of coil set and other deformities caused by internal residual stresses. But again, it should be borne in mind that, in performing the methods of the present invention, the surface conditioning apparatus **10** may be used in conjunction with other machines for flattening and leveling sheet metal, without departing from the scope of the present invention.

FIG. 3 is a schematic representation of still another in-line metal processing system in which the methods of the present invention may be practiced. Like the system depicted in FIG. 2, the system of FIG. 3 shows the surface conditioning apparatus **10** used in conjunction with the tension leveler **40**, but in this embodiment the surface conditioning apparatus **10** is positioned between the leveler portion **52** and the pull bridle **54** of the tension leveler **40**, rather than downstream of the pull bridle **54** as shown in FIG. 2. Aside from the location of the surface conditioning apparatus **10** relative to the components of the tension leveler **40**, the embodiment of FIG. 3 is generally similar to the embodiment of FIG. 2. When the surface conditioning apparatus **10** is located between the leveling rollers **60** and the pull bridle **54**, the surface conditioning apparatus **10** engages the metal sheet **46** (in a manner described hereinafter) while the metal sheet **46** is subjected to the tensile force between the drag and pull bridles **50** and **54**. While under this tension, the metal sheet **46** is in an extremely flat condition, which allows for best performance of the surface conditioning apparatus **10**. However, once again, the system depicted in FIG. 3 is intended to illustrate another preferred environment in

which the methods of the present invention may be practiced. Certainly, other sheet metal flattening and leveling machines could be used in connection with the surface conditioning apparatus **10** to perform the methods claimed herein, without departing from the scope of the present invention.

FIG. 4 is an enlarged view of certain key components of the surface conditioner **10**, and FIG. 5 is a top plan view of certain key components of the surface conditioner **10**. As shown in FIGS. 4 and 5, the surface conditioner **10** includes a rotating cleaning brush **70**, a plurality of coolant/lubricant sprayers **72**, and a back-up roller **74**. The cleaning brush **70** includes a mildly abrasive conditioning surface **76** having a generally cylindrical configuration.

It has been found that cleaning brushes manufactured by Minnesota Mining and Manufacturing (3M) under the name Scotch-Brite®, or their equivalent, are suitable for use in the surface conditioner **10** of the present invention. In these brushes, abrasive particles are bonded to resilient synthetic (e.g., nylon) fibers of the brush with a resin adhesive. The resilient brush fibers of the Scotch-Brite® product are of an open-web construction, which gives the fibers a spring-like action that conforms to irregular surfaces and prevents surface gouging. Scotch-Brite® brand cleaning brushes are available in a variety of grades of coarseness and fiber density, though suitable abrasive and non-abrasive cleaning brushes manufactured by others could be used without departing from the scope of the present invention. The inventor has determined that 3M's Scotch-Brite® brand finishing-cleaning brushes identified by 3M item number #048011-90626-3, SPR 22293A are suitable for use in practicing the methods of the present invention, though other brushes with other grades of coarseness and fiber density may also be suitable. The selection of other suitable brushes would be within the skill of one of ordinary skill in the art.

As shown in FIG. 4, the cleaning brush **70** is preferably positioned above the sheet metal strip **46** for engagement with a surface thereof. Preferably, the cleaning brush **70** is rotated in a direction against the movement of the strip through the surface conditioner **10** (clockwise as viewed in FIG. 4, with the strip **46** advancing from left to right). The backup roller **74** engages against the opposite surface of the strip **46** and applies a force equal and opposite to the downward force applied by the cleaning brush **70**. Preferably, the back-up roller **74** moves in the same direction as the strip **46** (clockwise as viewed in FIG. 4). The back-up roller **74** may be powered to assist in advancing the strip **46** through the surface conditioner **10**. It should be understood, however, that although FIGS. 4 and 5 depict only one cleaning brush **70** positioned for engagement with a top surface of the strip **46**, additional brushes positioned for engagement with the upper and/or lower surfaces of the strip may be used without departing from the scope of the invention.

Preferably, a spray bar **80** having a plurality of sprayer nozzles **72** is positioned just downstream of the cleaning brush **70**, with the sprayer nozzles **72** aimed generally toward the point of engagement of the cleaning brush **70** and the surface of the strip **46**. The sprayer nozzles **72** apply a coolant/lubricant, such as water, to the cleaning brush **70** during operation of the surface conditioner **10**. Preferably, the coolant/lubricant is applied at the rate of about 4 to 6 gallons per minute per 12" length of the cleaning brush **70**. This enhances performance of the surface conditioner **10** by producing a cooler running operation, while washing away cleaning by-products (scale and smut removed by the abra-

sive surface of the brush), and by extending the life of the cleaning brush 70. As shown in FIG. 5, the spray nozzles 72 are preferably positioned to apply the coolant/lubricant in an overlapping spray pattern so that, if one of the nozzles gets plugged, adjacent nozzles can maintain substantially complete coverage. While the spray bar 80 positioned just downstream of the cleaning brush 70 is important for proper performance, additional spray bars (not shown) may be added at other locations upstream and downstream of the cleaning brush 70 and back-up roller 74.

For optimum performance, the surface conditioner 10 requires a very flat surface. This is why the stretcher leveling machine 12 and tension leveling machines 40 shown in FIGS. 1-3 and described above are preferred. However, again, assuming a sufficiently flat surface can be achieved, other sheet metal flattening and leveling machines can be used in connection with the surface conditioning apparatus 10 to perform the methods of the present invention claimed herein.

Preferably, the various apparatus and environments described above are used to practice the present invention, which includes methods of removing iron oxide scale from processed sheet metal. FIG. 6 depicts a section of processed sheet metal 86 (e.g., hot rolled carbon steel) with layers of iron oxide scale on the surface, prior to surface conditioning according to the methods of the present invention. As shown in FIG. 6, the iron oxide scale generally comprises three layers: a wustite layer 88, a magnetite layer 90, and a hematite layer 92. The wustite layer 88 is bonded to a base metal substrate 94 of the processed sheet metal. The magnetite layer 90 is bonded to the wustite layer 88, and the hematite layer 92 is bonded to the magnetite layer 90. Note that the various layers shown in FIG. 6 are depicted in a manner that is easy to view; but FIG. 6 is not necessarily to scale. As explained above, in hot rolled carbon steel cooled from finishing temperatures above 1058° F. (570° C.), the oxide layer will typically comprise at least 50% wustite, as well as some magnetite and hematite, with the overall thickness of these three layers being about 0.5% of the total thickness of the steel sheet. Thus, for example, in  $\frac{3}{8}$ " hot rolled carbon steel, the overall thickness of the oxide layer will be about 0.002".

In general, a method of the present invention comprises conditioning a surface of the processed sheet metal 46 with the surface conditioning apparatus 10 by bringing the generally cylindrical conditioning surface 76 of the rotating cleaning brush 70 into engagement with the surface of the sheet metal 46. As the sheet metal 46 is advanced through the surface conditioning apparatus 10, the rotating cleaning brush 70 is rotated in the upstream direction against the downstream advancement of the length of sheet metal 46. This engagement of the brush 70 against the surface of the sheet metal 46 removes substantially all of the hematite layer 92 and magnetite layer 90 from the surface. In addition, the engagement of the brush 70 against the surface of the sheet metal 46 removes some (but not all) of the wustite layer 88 from the surface, so that a portion of the wustite layer 88 remains bonded to the base metal substrate 94 of the processed sheet metal, as shown in FIG. 7, which depicts a section of processed sheet metal 96 following surface conditioning according to the methods of the present invention. As with FIG. 6, note that the layers shown in FIG. 7 are not to scale. Again, in hot rolled carbon steel cooled from finishing temperatures above 1058° F. (570° C.), the overall thickness of the three oxide layers prior to surface conditioning in accordance with the present invention is about 0.5% of the total thickness of the steel sheet, and after

surface conditioning in accordance with the present invention, the thickness of the remaining wustite layer 88 much less than 0.5% of the total thickness. Preferably, at least 10% of the wustite layer 88 is removed from the surface of the sheet metal 46. More preferably, conditioning the surface of the processed sheet metal in this manner removes between 10% and 50% of the wustite layer 88 from the surface of the sheet metal 46. Even more preferably, the step of conditioning is performed in a manner to remove about 30% of the wustite layer 88 from the surface of the sheet metal 46, leaving a remaining layer of wustite. Limited research has shown that the remaining layer of wustite measures no more than about 0.001 inches in average thickness, but which preferably measures between about 0.00035 inches and 0.00085 inches in average thickness. Even more preferably, the remaining layer of wustite measures about 0.00055 inches in average thickness.

The hematite layer 92 and magnetite layer 90 are rather brittle, so the above-described mechanical brushing is very effective at removing all or substantially all of these layers. The removal of these layers has been confirmed by a napkin wipe test (e.g., wiping a napkin across the surface), which is considered standard process control. Once the surface has been conditioned in accordance with the methods of the present invention, a napkin wiped across the surface should not pick up any visually perceptible scale or smut. Also, as indicated above, this mechanical brushing also preferably removes about 30% of the tightly adhered wustite layer 88 from the surface of the sheet metal 46, leaving a layer of wustite bonded to the base metal substrate 94. It has been found that the remaining layer of wustite 88 is beneficial because it allows the conditioned surface of the sheet metal to withstand further oxidation. Limited research by the inventors herein has shown that this benefit occurs at least in part as a result of the mechanical brushing removing all or substantially all of the magnetite and hematite composition layers. With these layers removed, there is less available free iron to form a "red rust" oxide. Magnetite (chemically known as  $Fe_3O_4$ ) and hematite (chemically known as  $Fe_2O_3$ ) contain much more available iron atoms than the remaining wustite layer (chemically known as  $FeO$ ). It is also theorized that the process of mechanical brushing has a "smearing" effect on the remaining wustite layer, which may contribute to the sheet metal's ability to withstand further oxidation by making the remaining wustite layer more uniform and thereby reducing the likelihood of ambient oxygen and moisture reaching the base metal substrate 94. However, this theory has not been confirmed.

In another aspect of the present invention, a method of removing iron oxide scale from processed sheet metal comprises the steps of: providing a surface conditioning apparatus 10 having at least one rotating conditioning brush 70; and conditioning a surface of the processed sheet metal 46 by bringing the rotating conditioning brush 70 into engagement with the surface of the sheet metal 46 in a manner to remove some, but less than substantially all of the iron oxide scale from the surface so that a layer of wustite 88 remains bonded to a base metal substrate 94, and in a manner to smooth the surface. Preferably, the "smoothing" achieved by engagement of the rotating conditioning brush 70 with the surface of the sheet metal 46 is sufficient to reduce an arithmetic mean of distances of departure of peaks and valleys on the surface, measured from a mean center line, to less than 50 micro inches. More preferably, the smoothing achieved by the rotating conditioning brush 70 is sufficient to reduce the arithmetic mean of the distances of departure of peaks and valleys on the surface, measured from the mean center line, to between about 35 and 45 micro inches.

Surface roughness is measured with a profilometer, as is well known in the art, and is usually expressed as an "Ra" value in micro meters or micro inches. This Ra value represents the arithmetic mean of the departure of the peaks and valleys of the surface profile from a mean center line over several sampling lengths, and is therefore also sometimes referred to as a "center line average" (CLA). The lower the Ra value, the smoother the surface finish. Limited quantitative evidence exists demonstrating that hot rolled sheet metal surface conditioned in accordance with the methods of the present invention, as measured with a profilometer, has a lower (i.e., better) Ra value than that of typical hot rolled steel which has been pickled. In fact, limited research has shown that hot rolled sheet metal surface conditioned in accordance with the methods of the present invention has an Ra value that is comparable to or better than cold roll regular matte finish (which typically has an Ra value of between 40 and 60 micro inches).

The inventors herein have found that the surface of the remaining wustite layer **88** left by mechanical brushing in accordance with the present invention is relatively smooth (as indicated by the Ra values noted above) and requires minimal or no additional surface preparation prior to painting or other coating. It has been found that the painting characteristics of material surface conditioned in accordance with the present invention are as good or better than pickled material. To the eye, the surfaces are virtually indistinguishable, as both appear to be free of oxide scale. However, testing has shown that, over time, material surface conditioned in accordance with the present invention is better suited to resist further oxidation than similar material that has been pickled and oiled. Independent "salt spray tests" (which are standard in the industry) were conducted by Valspar Corporation, a reputable industrial paint manufacturer, and material that was stretcher leveled and then surface conditioned in accordance with the present invention was found to be substantially corrosion free after as long as 1000 hours of salt spray testing, whereas hot rolled steel that was pickled and oiled showed signs of further corrosion after as little as 144 hours of salt spray testing.

Again, it has been found that the layer of wustite **88** remaining after mechanical brushing in accordance with the methods of the present invention is beneficial because it inhibits further oxidation, due at least in part to the removal of all or substantially all of the magnetite and hematite composition layers, which leaves less available free iron to form "red rust" oxide. But in addition to this, and in addition to the smoothness benefits described above, mechanical brushing in accordance with the methods of the present invention is preferable to pickling and oiling because there is no need to remove the oil before coating; hydrochloric acid (an environmentally hazardous chemical that has special storage and disposal restrictions) is not used; and there is no oil to interfere with manufacturing processes, such as welding.

In view of the foregoing, it will be seen that the several advantages of the invention are achieved and attained. The embodiments were chosen and described in order to best explain the principles of the invention and its practical application to thereby enable others skilled in the art to best utilize the invention in various embodiments and with various modifications as are suited to the particular use contemplated. However, as various modifications could be made in the invention described and illustrated without departing from the scope of the invention, it is intended that all matter contained in the foregoing description or shown in

the accompanying Figures shall be interpreted as illustrative rather than limiting. Thus, the breadth and scope of the present invention should not be limited by any of the above-described exemplary embodiments, but should be defined only in accordance with following claims appended hereto and their equivalents.

What is claimed is:

1. A method of removing iron oxide scale from processed sheet metal, wherein the iron oxide scale generally comprises a wustite layer that is bonded to a base metal substrate of the processed sheet metal, a magnetite layer that is bonded to the wustite layer, and a hematite layer that is bonded to the magnetite layer, the method comprising the steps of:
  - 15 providing a surface conditioning apparatus having at least one surface conditioning member; and
  - conditioning a surface of the processed sheet metal with the surface conditioning apparatus by bringing the at least one surface conditioning member into engagement with the surface of the sheet metal in a manner to remove substantially all of the hematite and magnetite layers from the surface, and in a manner to remove less than substantially all of the wustite layer from the surface so that a portion of the wustite layer remains bonded to the base metal substrate of the processed sheet metal.
2. The method of claim 1 wherein the step of conditioning the surface of the processed sheet metal includes removing at least 10% of the wustite layer from the surface of the sheet metal.
3. The method of claim 2 wherein the step of conditioning the surface of the processed sheet metal includes removing between 10% and 50% of the wustite layer from the surface of the sheet metal.
- 35 4. The method of claim 3 wherein the step of conditioning the surface of the processed sheet metal includes removing about 30% of the wustite layer from the surface of the sheet metal.
5. The method of claim 1 wherein the step of conditioning the surface of the processed sheet metal includes removing an amount of the wustite layer from the surface so that a remaining layer of wustite measures no more than about 0.001 inches in average thickness.
- 40 6. The method of claim 5 wherein the step of conditioning the surface of the processed sheet metal includes removing an amount of the wustite layer from the surface so that a remaining layer of wustite measures between about 0.00035 inches and 0.00085 inches in average thickness.
7. The method of claim 1 wherein the at least one surface conditioning member is a rotating conditioning member having a generally cylindrical conditioning surface, and wherein the step of conditioning the surface of the processed sheet metal with the surface conditioning apparatus includes bringing the generally cylindrical conditioning surface of the rotating conditioning member into engagement with the surface of the sheet metal.
- 50 8. The method of claim 7 wherein the at least one rotating conditioning member comprises a brush having a plurality of resilient fibers.
9. The method of claim 7 further comprising the step of advancing a length of the sheet metal through the surface conditioning apparatus in a downstream direction, and wherein the step of conditioning the surface of the processed sheet metal by bringing the at least one rotating conditioning member into engagement with the surface of the sheet metal is performed as the length of the sheet metal is advanced through the surface conditioning apparatus.

**11**

**10.** The method of claim **9** wherein the step of conditioning the surface of the processed sheet metal by bringing the at least one rotating conditioning member into engagement with the surface of the sheet metal includes rotating the at least one rotating conditioning member in an upstream direction against the downstream advancement of the length of sheet metal.

**11.** The method of claim **1** wherein the surface conditioning apparatus further comprises at least one coolant sprayer and wherein the step of conditioning the surface of the sheet metal with the surface conditioning apparatus includes applying a coolant to one of the rotating conditioning member and the surface with the at least one coolant sprayer.

**12.** The method of claim **11** further comprising the step of washing away scale removed from the surface of the sheet metal by applying the coolant to one of the rotating conditioning member and the surface with the at least one coolant sprayer.

**13.** The method of claim **1** wherein the step of conditioning the surface of the processed sheet metal includes bringing the at least one surface conditioning member into engagement with the surface of the sheet metal in a manner to reduce an arithmetic mean of distances of departure of peaks and valleys on the surface, measured from a mean center line, to less than 50 micro inches.

**14.** The method of claim **13** wherein the step of conditioning the surface of the processed sheet metal includes bringing the at least one rotating conditioning member into engagement with the surface of the sheet metal in a manner to reduce the arithmetic mean of the distances of departure of peaks and valleys on the surface, measured from the mean center line, to between about 35 and 45 micro inches.

**15.** A method of removing iron oxide scale from processed sheet metal, wherein the iron oxide scale generally comprises a wustite layer that is bonded to a base metal substrate of the processed sheet metal, a magnetite layer that

5

10

15

20

25

35

**12**

is bonded to the wustite layer, and a hematite layer that is bonded to the magnetite layer, the method comprising the steps of:

providing a surface conditioning apparatus having at least one rotating conditioning member with a generally cylindrical conditioning surface; and

conditioning a surface of the processed sheet metal with the surface conditioning apparatus by bringing the generally cylindrical conditioning surface of the at least one surface conditioning member into engagement with the surface of the sheet metal in a manner to remove substantially all of the hematite and magnetite layers from the surface, and in a manner to remove less than substantially all of the wustite layer from the surface so that a portion of the wustite layer remains bonded to the base metal substrate of the processed sheet metal.

**16.** The method of claim **15** wherein the step of conditioning the surface of the processed sheet metal includes bringing the generally cylindrical conditioning surface of the at least one surface conditioning member into engagement with the surface of the sheet metal in a manner to reduce an arithmetic mean of distances of departure of peaks and valleys on the surface, measured from a mean center line, to less than 50 micro inches.

**17.** The method of claim **16** wherein the step of conditioning the surface of the processed sheet metal includes bringing the generally cylindrical conditioning surface of the at least one surface conditioning member into engagement with the surface of the sheet metal in a manner to reduce an arithmetic mean of distances of departure of peaks and valleys on the surface, measured from a mean center line, to between about 35 and 45 micro inches.

\* \* \* \* \*